

[54] IMINOPHENOLS AS FROTH FLOTATION  
REAGENTS FOR METALLIC ORES

[76] Inventor: Vojislav Petrovich, 1929 W. Schiller  
St., Chicago, Ill.  
[22] Filed: Apr. 30, 1974  
[21] Appl. No.: 465,412

[52] U.S. Cl. .... 209/166  
[51] Int. Cl.<sup>2</sup> .... B03D 1/02  
[58] Field of Search..... 209/166, 167

[56] References Cited

UNITED STATES PATENTS

|           |         |                |           |
|-----------|---------|----------------|-----------|
| 2,272,489 | 2/1942  | Ulrich .....   | 260/239 E |
| 2,296,226 | 9/1942  | Ulrich .....   | 260/239 E |
| 2,414,199 | 1/1947  | Gutzeit .....  | 209/166   |
| 3,056,498 | 10/1962 | De Grote ..... | 209/166   |
| 3,425,549 | 2/1969  | Dickson .....  | 209/166   |
| 3,819,048 | 6/1974  | Weimer .....   | 209/166   |

Primary Examiner—Robert Halper

[57] ABSTRACT

A froth flotation method for the recovery of iron, copper, cobalt, nickel, and vanadium minerals from their ores over silica, alumino, and ferromagnesian silicates, which comprises subjecting the comminuted ore of aforesaid metals to froth flotation process in the presence of an effective amount of iminophenols such as methyliminodihydroxybenzoic acid, methyliminocresolcresylic acid, methyliminocresol adduct of polyethylene glycol, the indicated compounds provide selectivity and recovery of metal values of iron, copper, cobalt, nickel, and vanadium from their oxide, silicate, sulfide, arsenide, and antimonide ores in an enriched froth concentrate of the said minerals, leaving a tailings poor in these minerals.

3 Claims, No Drawings

# IMINOPHENOLS AS FROTH FLOTATION REAGENTS FOR METALLIC ORES

This invention relates to the concentration of metal values from their ores. Particularly, it relates to the use of iminophenols as flotation reagents to effect a separation of metal values in ores from gangue. More particularly, it relates to the use of aryl iminophenols as froth flotation reagents for oxide ores of iron, oxide, silicate, sulfide ores of copper, oxide, silicate, sulfide, arsenide, and antimonide ores of nickel, as well as of cobalt, and vanadate of heavy metals.

The special feature of this invention using iminophenols is in the nonfloating of minerals with divalent iron, i.e., the common sulfide of iron as is pyrite, arsenopyrite, furthermore, ferromagnesian silicates and the like minerals, as are garnet, biotite, chlorite, hornblende, augite, forsterite, fayalite, talc, talcy materials, and the like minerals.

## THE PREFERRED EMBODIMENTS

The preferred embodiments of collectors of this invention are as follows:

Methyl-imino-di-hydroxybenzoic acid of the formula:



Methylinocresolcresolic acid of the formula:



Methylinocresol adduct of polyethylene glycol of the formula:



wherein  $n$  is an integer from 5 to 15.

The said iminophenol acting as froth flotation collectors, function through the conjunctive action of phenolic hydroxide and imine nitrogen  $=N-$  attached directly to the benzene nucleus; both groups are in alfa position to each other. The active group of this constitution, i.e., of a phenolic hydroxyl and an imine nitrogen are the only promoting groups and essential part of the flotation reagent with collecting power. All other grouping parts, i.e., the adduct of alcohol hydrocarbon group, the adduct of cresolic acid are auxiliary groupings, which aid in the bubble formation, an essentially secondary property.

The active groups are hydrophilic until promoting takes place and aid in solubility of the reagents. After promoting, the hydrophilic property of the active group is lost, in which case the hydrophilic part outside the active group begins to form bubbles due to its constitu-

tion. Thus, these iminophenols function as complete froth flotation collectors.

Although some classes of amines are known to be helpful in the recovery of metal values by flotation, applicant has not been able to find a teaching that the iminophenols are capable of acting as flotation collectors. However, applicant has found them to be remarkably well suited to flotation of certain types of ores. In fact, applicant has discovered that the iminophenols are capable of collecting iron, cobalt, nickel, copper, and vanadium ores without a preflotation treatment.

Good recoveries of said metal values in respective minerals are obtained if the reagents of the present invention are used in a circuit having a pH about 8 to 12.

15 Further advantage of this invention resides in the fact that no specific frothing agents are to be employed, since the products of this invention develop sufficient froth to be good promoter and frother at the same time, which adds in the over-all economy and operativity of 20 the process.

The further advantage of this invention resides in the feasibility of recycling the processed water after desliming by cycloning, which would enable big savings in alkalies and ammonia.

25 Accordingly, a principal object of this invention is to provide a new class of froth flotation reagents.

A further object of this invention is to provide flotation reagents with collecting and frothing properties for collecting iron oxide ores, copper oxide, silicate, and sulfide ores, nickel as well as cobalt oxide, silicate, sulfide, arsenide, and antimonide ores, and the vanadates of heavy metals.

30 A still further object is to disclose the novel agents for handling ores wherein the use of activation step of any kind is unnecessary. I have discovered that most gangue minerals are unaffected by the collector of this invention. Hence a method for obtaining a highly selective concentration of the desired metal values is provided.

35 The collectors of the invention, which function by chemical reaction with the ore treated have complexing and presumably chelating ability at the very surface of mineral or portion of surface of the mineral particle of the ore treated. It is obvious that the polar part, i.e., the complexing or chelating groups, i.e., the phenolic hydroxyl and the imine-nitrogen of the reagent are oriented towards the ore particle, while the hydroxyhydrocarbon or alkanol part of the reagent is oriented outward from said particle. Thus the attachment of 40 these organic complexing and chelating ingredients to the ore particles form a water repellent surface, or barrier, around at least a part of the surface of the ore particle and thereby facilitates the formation of the froth when the ore slurry is agitated in the presence of air.

50 The froth flotation of the present invention is carried out in accordance with good flotation practice and usually, though not always, involves flotation in rougher cells, followed by one or several cleanings of the rougher concentrate. The reagents are effective in small amounts and the promotion is sufficiently persistent so that it is feasible to carry out the rougher and cleaner flotation with a single addition of the reagents at the beginning of the operation. On the other hand, it is sometimes advantageous to use stage addition of reagents. Pulp densities are in general the same as in other applications of froth flotation practice, i.e., about 15 to 60 30 percent of solids by weight.

The flotation plant practice applying the inventor's method by serving the iminophenols for the recovery of metal values, floating the hereinbefore said ores and minerals of iron, cobalt, nickel, copper, and vanadium with aryl or aralkyl iminophenols having collecting and frothing properties, the ore is crushed, milled and sized to at least about 80 to 120 mesh standard sieve, which depends on the particular ore treated. Milling to finer sizes is preferable. The crushed and sized ore is pulped and as a mineral slurry is ready for treatment in the flotation plant equipment, i.e., by passing through the conditioner where the collector is added. From the conditioner the pulp is pumped in the receiving box of the first stage or the main flotation bank. In the main flotation bank the froth produced by agitation and aeration is skimmed or is overflowing in the usual manner. In most cases it is advantageous to use multiple stage flotation process to treat the underflow or partially metal value barren pulp to increase the degree of separation or to enhance the grade of recovery. Also, the use of varying amounts of emulsifiers, dispersants, and depressants etc. in different stages may be used to advantage to obtain the highest yield and best separation.

Having disclosed the novel collectors of this invention as well as the handling of the mineral slurry, I have to say the final object of this invention is to provide a method for the flotation recovery of minerals contain-

5  
10  
15  
20  
25

sieve. Transferring the sized flotation feed in the flotation machine, various amounts of said iminophenols for collecting purposes were added. After this step, the pulp of mineral slurry was conditioned for 5 minutes. The amounts of collector, as well as ammonia to make a pH of about 10 to 11, are indicated in the accompanying table. Before skimming of the rougher concentrate the pulp of mineral slurry was conditioned and aerated for three to five minutes. The rougher concentrates were skimmed from about five to ten minutes and afterwards cleaned with processed water.

The flotation test of sized sample of ullmannite and chloanthite for determination of floatability of nickel ores; and of smaltite and linnaeit for determination of floatability of cobalt ores; as well as of carnotite for determination of floatability of vanadium ores, were accomplished in a 50 grams flotation cell. The feed were prepared with 5 grams of a mixture of ullmannite and chloanthite, as well as 5 grams of a mixture of smaltite and linnaeite, and 45 grams of a mixture of pyrite, arsopyrite, pyrrhotite, and galena as gangue material respectively, as well as 45 grams of a mixture of crystalline schist material and sandstone as gangue material with 5 grams of carnotite. The addition of reagents was done dropwise. The recovery of ullmannite-chloanthite; smaltite-linnaeite; and of carnotite was obtained by microscopic count.

| Ore treated                                 | Collector pound per ton                                     | NH <sub>3</sub> | Assay Feed                        | of Conc.          | products Recovery |
|---------------------------------------------|-------------------------------------------------------------|-----------------|-----------------------------------|-------------------|-------------------|
| Example 1<br>Hematite                       | Methyliminocresolcresylic acid<br>0.6                       | 0.3             | Fe %<br>32.2                      | Fe %<br>65.8      | Fe %<br>92.0      |
| Example 2<br>Copper sulfide                 | Methylimino-di-hydroxybenzoic acid<br>0.35                  | 0.3             | Cu %<br>2.8                       | Cu %<br>23.8      | Cu %<br>94.1      |
| Example 3<br>copper carbonate<br>Malachite  | Methyl iminocresol adduct<br>of polyethylene glycol<br>0.35 | 0.3             | Cu %<br>1.8                       | Cu %<br>43.2      | Cu %<br>94.4      |
| Example 4<br>copper silicate<br>Chrysocolla | Methylimino-di-hydroxybenzoic acid<br>0.35                  | 0.3             | Cu %<br>2.2                       | Cu %<br>30.8      | Cu %<br>91.6      |
| Example 5<br>Ni-silicate<br>Garnierite      | Methylimino-di-hydroxybenzoic acid<br>0.20                  | 0.3             | Ni %<br>2.2                       | Ni %<br>10.4      | Ni %<br>94.2      |
| Example 6<br>Ullmannite<br>Chloanthite      | Methyliminocresolcresylic acid<br>—                         | —               | Ni %<br>—<br>by microscopic count | Ni %<br>—<br>88.0 | Ni %<br>—<br>88.0 |
| Example 7<br>Smaltite<br>Linnaeite          | Methyliminocresolcresylic acid<br>—                         | —               | Co %<br>—<br>by microscopic count | Co %<br>—<br>86.0 | Co %<br>—<br>86.0 |
| Example 8<br>Carnotite                      | Methyliminocresolcresylic acid<br>—                         | —               | V %<br>—<br>by microscopic count  | V %<br>—<br>92.0  | V %<br>—<br>92.0  |

ing iron, cobalt, nickel, copper, and vanadium.

The above discussion as well as the disclosure illustrate my invention in a broad and general way; for a detailed illustration thereof the examples of the preferred embodiments of flotation practice are set forth below.

The procedure in performing the laboratory examples for iron, nickel, and copper ores was of the same manipulation as follows: specular hematite, copper sulfide, copper silicate, copper carbonate, and nickel silicate ore, the feed was sized to pass 100 mesh standard

60  
65

It is to be understood that the foregoing detailed discussion is for the purpose of illustration only, and it is not intended as being limiting to the spirit or scope of the appended claims.

What I claim is:

1. A method of beneficiating ores selected from the groups consisting of oxide of iron, oxide, silicate, and sulfide of copper, oxide, silicate, sulfide, arsenide, and antimonide of nickel, oxide, sulfide, arsenide, and antimonide of cobalt, the vanadate of heavy metals by froth

flotation process to produce a froth concentrate of desired metal values which comprises effecting the froth flotation of the said ores and minerals in the presence of methyliminodihydroxybenzoic acid as collector in a pulp of mineral slurry having a pH of 8 to 12; and recovering the desired metal value in an enriched froth concentrate, leaving a tailings poor in the desired metal value.

2. A method of beneficiating ores selected from the groups consisting of oxide of iron, oxide, silicate, and sulfide of copper, oxide, silicate, sulfide, arsenide, and antimonide of nickel, oxide, sulfide, arsenide, and antimonide of cobalt, the vanadate of heavy metals by froth flotation process to produce a froth concentrate of desired metal values which comprises effecting the froth flotation of the said ores and minerals in the presence of methyliminocresolcresylic acid as collector in a pulp of mineral slurry having a pH of 8 to 12; and recovering

the desired metal value in an enriched froth concentrate, leaving a tailings poor in the desired metal value.

3. A method of beneficiating ores selected from the groups consisting of oxide of iron, oxide, silicate, and sulfide of copper, oxide, silicate, sulfide, arsenide, and antimonide of nickel, oxide, sulfide, arsenide, and antimonide of cobalt, the vanadate of heavy metals by froth flotation process to produce a froth concentrate of desired metal values which comprises effecting the froth flotation of the said ores and minerals in the presence of methyliminocresol adduct of polyethylene glycol as collector, said adduct having 5 to 15 methyl groups in said polyethylene glycol, the flotation being effected in a pulp of mineral slurry having a pH of 8 to 12; and recovering the desired metal value in an enriched froth concentrate, leaving a tailings poor in the desired metal value.

\* \* \* \* \*

20

25

30

35

40

45

50

55

60

65

UNITED STATES PATENT OFFICE  
CERTIFICATE OF CORRECTION

Patent No. 3,891,545 Dated June 24, 1975

Inventor(s) Vojislav Petrovich

It is certified that error appears in the above-identified patent and that said Letters Patent are hereby corrected as shown below:

Column 1, lines 45 to 49, the formula should appear as shown below:



Signed and Sealed this  
twenty-fifth Day of November 1975

[SEAL]

Attest:

RUTH C. MASON  
Attesting Officer

C. MARSHALL DANN  
Commissioner of Patents and Trademarks